

## UNITED STATES PATENT OFFICE

THOMAS H. MCKEOWN, OF METUCHEN, NEW JERSEY, ASSIGNOR, BY MESNE ASSIGNMENTS, TO THE ROESSLER & HASLACHER CHEMICAL COMPANY, A CORPORATION OF DELAWARE

## OPACIFIER FOR ENAMELS

No Drawing. Application filed January 12, 1928. Serial No. 246,398.

This invention relates to the manufacture of white vitreous enamels and has for its object the development of an enamel utilizing a relatively inexpensive opacifier which will 5 impart to the enamel a desirable white color. A further object is to provide such an enamel particularly suited for dry process application on cast metal, such as cast iron or steel.

My invention consists in providing enamel mixtures containing sodium antimonate and tin oxide as opacifier. I have tried various mixtures of sodium antimonate and tin oxide in a number of varied formulae, but I have found that the best results are secured if the 10 two constituents are present in a more or less restricted ratio to each other. I have found that the sodium antimonate-tin oxide ratios should be approximately 3:1. If this ratio is altered in either direction the enamel 15 in which it is used does not have the desired opacity and physical properties. I have found that in the enamels of my invention this 3:1 mixture can be utilized in amounts sufficient to give desired opacity and color, 20 and still not render the enamel brittle or increase its tendency to chip off, i. e. the proper cubical expansion of the enamel necessary to secure the proper adherence to the iron 25 or steel under temperature changes can be obtained even with high amounts of this opacifier.

I have further discovered that to secure the proper adherence and other desirable qualities in such enamels several components 30 must be used in more or less definite proportions. The following example gives these components in the preferred proportions and the variable allowances which may be made in the components to secure small variations 35 in the expansion coefficient to conform to the metal. The individual coefficients of expansion of the components are given in the literature so that having the basic formula given here below the desired composition can be 40 made up to fit any particular cast metal.

In this example and in the appended claims my opacifier is referred to as "antimony-tin opacifier", and the amount required denotes the amount of 3:1 mixture used.

| Dry process cast iron enamel             |                        | 50                       |    |
|------------------------------------------|------------------------|--------------------------|----|
|                                          | Preferred frit formula | Variable frit allowances | 55 |
| Feldspar (parts by weight)               | 37.0                   | 35 to 39                 |    |
| Borax (parts by weight)                  | 13.0                   | 11 to 14                 |    |
| Soda nitre (parts by weight)             | 2.5                    | 2 to 3                   |    |
| Soda ash (parts by weight)               | 7.0                    | 5 to 8                   |    |
| Cryolite (parts by weight)               | 4.0                    | 3 to 6                   |    |
| Fluorspar (parts by weight)              | 6.0                    | 5 to 7                   |    |
| Whiting (parts by weight)                | 3.0                    | 1 to 4                   |    |
| Red lead (parts by weight)               | 15.0                   | 10 to 15                 | 60 |
| Zinc oxide (parts by weight)             | 4.5                    | 3 to 7                   |    |
| Antimony-tin opacifier (parts by weight) | 8.0                    | 4 to 12                  |    |

The powdered materials of this formula are mixed by hand or mechanically, and then fused; the melt is dropped into water to cool and shatter after which it is placed in the ball mill and ground together to a fineness best suited for the particular method of application to be used; this fineness will be generally between about 30-70 mesh.

In using this enamel on cast iron a slush or binding coat is first applied to the article. This undercoat may be any of the coating compositions suited for the articles. Such a slush coat for cast metal is formed by fusing together feldspar, flint, borax, red lead and saltpeter to form a frit in grinding this with water, clay and further amounts of feldspar and flint. This mixture is applied to the casting and then fired at a temperature of about 875° C.; the casting is then withdrawn from the furnace, and the powdered enamel dusted on the hot casting after which the casting is again fired. Several applications of the enamel can thus be made depending on the thickness of enamel desired. As noted above the maturing temperature of this enamel is about 850° C. A period of about 5 minutes at this temperature is usually satisfactory.

When thus burned the above enamel has the following empirical formula when calculated on a basis wherein the sum of the sodium, potassium, calcium, lead and tin oxides is equal to one.

|                                | Mols. |
|--------------------------------|-------|
| Na <sub>2</sub> O              | 0.407 |
| K <sub>2</sub> O               | 0.068 |
| CaO                            | 0.252 |
| Al <sub>2</sub> O <sub>3</sub> | 0.171 |
| B <sub>2</sub> O <sub>3</sub>  | 0.149 |
| Sb <sub>2</sub> O <sub>3</sub> | 0.030 |
| SiO <sub>2</sub>               | 0.970 |
| SnO <sub>2</sub>               | 0.030 |
| F <sub>2</sub>                 | 0.174 |
| PbO                            | 0.149 |
| ZnO                            | 0.123 |

The coefficient of expansion obtained with the preferred formula is  $365.4 \times 10^{-7}$ .

The variable compositions allowable in this flux will result in fluxes having a variable composition by weight approximately as follows:

|    |                                |           |
|----|--------------------------------|-----------|
| 25 | Na <sub>2</sub> O              | 9 to 12.5 |
|    | K <sub>2</sub> O               | 2.5 to 3  |
|    | CaO                            | 4 to 8    |
|    | Al <sub>2</sub> O <sub>3</sub> | 7 to 9    |
|    | B <sub>2</sub> O <sub>3</sub>  | 4 to 5    |
| 30 | Sb <sub>2</sub> O <sub>3</sub> | 2 to 6    |
|    | SiO <sub>2</sub>               | 24 to 28  |
|    | SnO <sub>2</sub>               | 1 to 3    |
|    | F <sub>2</sub>                 | 2 to 4    |
|    | PbO                            | 10 to 15  |
| 35 | ZnO                            | 3 to 7    |

In the above formulæ it will be noted that the opacifier allowances cover a wide range; the actual amount to be used depends on the opacity desired.

While I have explained the opacifier as being a definite mixture of the two materials, I have found that it is not necessary to actually mix or grind the antimonate and tin oxide together before adding them to the enamel. I have found that the opacifying results are equally well secured if, for example, the two were mixed prior to the addition of the enamel, or whether they were added separately, the only requirement being that the ratio approximately be maintained. Regardless of how the two materials are added any deviation from the ratio 3:1 is immediately apparent by a change in the appearance and properties of the enamel. It can be seen from the above I do not wish to be limited to the manner of adding my opacifying mixtures to the enamel. The sodium antimonate of my antimony tin opacifier may be supplied by pure sodium antimonate as such, or I may use the material commonly known in the art as leukonin which consists chiefly of sodium antimonate, and therefore in the appended claims, I wish it understood that sodium antimonate is intended to cover such

mixtures, and the term "antimony tin" opacifier is intended to cover such materials as leukonin in combination with tin oxide as well as the pure material.

Formulæ suited for sheet steel and wet process cast iron enameling embodying my invention are given in my copending applications, Serial No. 246,397 and Serial No. 246,399 respectively, filed of even date here-with.

Claims:

1. An enamel composition comprising:

|                              | Parts by weight |    |
|------------------------------|-----------------|----|
| Feldspar                     | 35 to 39        | 70 |
| Borax                        | 11 to 14        | 80 |
| Soda nitre                   | 2 to 3          |    |
| Soda ash                     | 5 to 8          |    |
| Cryolite                     | 3 to 6          |    |
| Fluorspar                    | 5 to 7          |    |
| Whiting                      | 1 to 4          | 85 |
| Red lead                     | 10 to 15        |    |
| Zinc oxide                   | 3 to 7          |    |
| Antimony-tin opacifier (3:1) | 4 to 12         |    |

2. An enamel composition comprising:

|                              | Parts by weight |    |
|------------------------------|-----------------|----|
| Feldspar                     | 37.0            |    |
| Borax                        | 13.0            |    |
| Soda nitre                   | 2.5             | 95 |
| Soda ash                     | 7.0             |    |
| Cryolite                     | 4.0             |    |
| Fluorspar                    | 6.0             |    |
| Whiting                      | 3.0             |    |
| Red lead                     | 15.0            |    |
| Zinc oxide                   | 4.5             |    |
| Antimony-tin opacifier (3:1) | 8.0             |    |

3. A fired enamel having the following empirical formula:

|                                | Mols. |     |
|--------------------------------|-------|-----|
| Na <sub>2</sub> O              | 0.407 | 105 |
| K <sub>2</sub> O               | 0.068 |     |
| CaO                            | 0.252 |     |
| Al <sub>2</sub> O <sub>3</sub> | 0.171 |     |
| B <sub>2</sub> O <sub>3</sub>  | 0.149 |     |
| Sb <sub>2</sub> O <sub>3</sub> | 0.030 | 110 |
| SiO <sub>2</sub>               | 0.970 |     |
| SnO <sub>2</sub>               | 0.030 |     |
| F <sub>2</sub>                 | 0.174 |     |
| PbO                            | 0.149 |     |
| ZnO                            | 0.123 | 115 |

4. A fired enamel having a composition by weight approximately as follows:

|                                |           |     |
|--------------------------------|-----------|-----|
| Na <sub>2</sub> O              | 9 to 12.5 | 120 |
| K <sub>2</sub> O               | 2.5 to 3  |     |
| CaO                            | 4 to 8    |     |
| Al <sub>2</sub> O <sub>3</sub> | 7 to 9    |     |
| B <sub>2</sub> O <sub>3</sub>  | 4 to 5    |     |
| Sb <sub>2</sub> O <sub>3</sub> | 2 to 6    | 125 |
| SiO <sub>2</sub>               | 24 to 28  |     |
| SnO <sub>2</sub>               | 1 to 3    |     |
| F <sub>2</sub>                 | 2 to 4    |     |
| PbO                            | 10 to 15  |     |
| ZnO                            | 3 to 7    | 130 |

wherein sodium antimonate and tin oxide are utilized in the requisite amount in the preparation of the composition for firing and in the ratio to each other of 3 to 1.

5 Signed at Perth Amboy, in the county of Middlesex and State of New Jersey, this tenth day of January, A. D. 1928.

THOMAS H. McKEOWN.

10

15

20

25

30

35

40

45

50

55

60

65